

## UNITED STATES PATENT OFFICE

TALMAGE B. WEAVER, OF MITCHELL, SOUTH DAKOTA

## PRESSING CLOTH

No Drawing.

Application filed October 8, 1927. Serial No. 225,020.

This invention relates to a pressing cloth of the type employed when pressing suits and other garments in order to prevent danger of scorching the material from which the 5 garment is made or causing cloth, such as serge, to become shiny.

One object of the invention is to provide a cloth impregnated with a dressing which will cause an iron to slide easily over the cloth 10 while pressing and also prevent the cloth from absorbing too much water when damped before being applied to the garment to be pressed.

Another object of the invention is to impregnate the cloth with a dressing which will serve to some extent to confine steam generated by the hot pressing iron between the cloth and the garment and thereby permit the 15 garment to be pressed in a very efficient manner.

Another object of the invention is to so apply the dressing to the cloth that it will be evenly distributed and excess dressing removed so that there will be no danger of the 20 garment being stained or otherwise soiled by the dressing when the cloth is in use.

The pressing cloth constituting the subject-matter of this invention consists of a strip of closely woven fabric and preferably 25 heavy muslin of a close fine weave is employed. This strip is cut the proper length and width for convenient use and the edges are hemmed to prevent fraying. After the strip of cloth has been cut and hemmed, it 30 is boiled in water and thoroughly rinsed to remove sizing and then dipped into a dressing consisting of a mixture of melted beeswax and gasoline. Preferably fifteen parts of gasoline and one part of beeswax are employed to form the dressing. After the cloth 35 has been dipped into the dressing and is thoroughly saturated, it is placed in a centrifugal extractor which rotates at a high rate of speed and the centrifugal force created removes 40 most of the excess dressing from the cloth. The cloth is then passed between heated rollers which serve to evenly distribute the dressing throughout the cloth and after being passed through the rollers the cloth is 45 placed in a heated dry room and left therein

until the gasoline remaining in the cloth has entirely evaporated and the cloth is deodorized. After the cloth is removed from the drying room, it is dipped into warm water and again placed in the centrifugal 55 extractor and after being removed from the extractor the cloth is passed through a heated mangle subjected to heavy pressure together with a strip of preferably white paper of an absorbent nature. The paper is placed 60 beneath the cloth when passed through the mangle and will serve to absorb any dressing which may be expressed from the cloth. This prevents any danger of too much dressing remaining in the cloth and causing a garment formed of light silk or thin cloth to be 65 stained or otherwise soiled while being pressed.

When the pressing cloth is in use, it is first dipped in water and wrung out to remove excess water therefrom and is then placed upon the garment to be pressed and the pressing operation carried out with a hot iron in the usual manner. Since the cloth 70 is impregnated with beeswax, the iron will 75 slide very easily across the cloth and in view of the fact that the wax fills the pores of the cloth steam generated between the cloth and garment will to a certain extent be confined and cause the garment to be pressed in a 80 very efficient manner. If desired, the dry cloth can be applied to the garment and after being sponged lightly ironed in the usual manner.

Having thus described the invention, I 85 claim:

1. A method of forming a pressing cloth consisting of providing a strip of fabric, immersing the fabric in boiling water and rinsing to remove sizing therefrom, dipping the strip into a dressing consisting of gasoline and melted beeswax, removing most of the excess dressing, distributing the dressing throughout the strip while subjecting the strip to heat and pressure, allowing excess gasoline to evaporate from the strip, dipping the strip in warm water and removing surplus moisture therefrom, laying a sheet of absorbent material upon the strip, and subjecting the sheet and the strip to heat and 90
2. A method of forming a pressing cloth consisting of providing a strip of fabric, immersing the fabric in boiling water and rinsing to remove sizing therefrom, dipping the strip into a dressing consisting of gasoline and melted beeswax, removing most of the excess dressing, distributing the dressing throughout the strip while subjecting the strip to heat and pressure, allowing excess gasoline to evaporate from the strip, dipping the strip in warm water and removing surplus moisture therefrom, laying a sheet of absorbent material upon the strip, and subjecting the sheet and the strip to heat and 95
3. A method of forming a pressing cloth consisting of providing a strip of fabric, immersing the fabric in boiling water and rinsing to remove sizing therefrom, dipping the strip into a dressing consisting of gasoline and melted beeswax, removing most of the excess dressing, distributing the dressing throughout the strip while subjecting the strip to heat and pressure, allowing excess gasoline to evaporate from the strip, dipping the strip in warm water and removing surplus moisture therefrom, laying a sheet of absorbent material upon the strip, and subjecting the sheet and the strip to heat and 100

high pressure whereby the remainder of the excess dressing will be removed therefrom.

2. A method of forming a pressing cloth consisting of providing a strip of fabric free from sizing, impregnating the fabric with a dressing consisting of gasoline and melted beeswax and extracting most of the excess dressing therefrom, subjecting the strip to heated pressing means to evenly distribute the dressing, allowing excess gasoline to evaporate from the strip, dipping the strip in warm water and then extracting the water, laying a sheet of absorbent material upon the strip, and subjecting the sheet and strip to heat and pressure whereby the remainder of the excess dressing will be removed from the strip.
3. A method of forming a pressing cloth consisting of providing a strip of fabric free from sizing, impregnating the fabric with a dressing consisting of gasoline and melted beeswax and evenly distributing the dressing and allowing excess gasoline to evaporate therefrom, dipping the dressed strip in water and then extracting the water, and finally removing excess dressing from the strip.

In testimony whereof I affix my signature.  
TALMAGE B. WEAVER [l. s.]

30

35

40

45

50

55

60

65